

# United States Patent [19]

Wiedemann

[11]

4,390,609

[45]

Jun. 28, 1983

[54] ELECTROPHOTOGRAPHIC RECORDING MATERIAL WITH ABRASION RESISTANT OVERCOAT

[75] Inventor: Wolfgang Wiedemann, Geisenheim, Fed. Rep. of Germany

[73] Assignee: Hoechst Aktiengesellschaft, Frankfurt am Main, Fed. Rep. of Germany

[21] Appl. No.: 291,050

[22] Filed: Aug. 7, 1981

[30] Foreign Application Priority Data

Aug. 30, 1980 [DE] Fed. Rep. of Germany ..... 3032774

[51] Int. Cl.<sup>3</sup> ..... G03G 5/14

[52] U.S. Cl. ..... 430/58; 430/66;  
430/67

[58] Field of Search ..... 430/56, 58, 59, 66,  
430/67, 89, 96

[56] References Cited

U.S. PATENT DOCUMENTS

2,901,348 8/1959 Dessauer et al. ..... 430/64 X  
3,140,174 7/1964 Clark .....  
3,810,759 5/1974 Stahr et al. ..... 430/56 X  
3,870,516 3/1975 Smith et al. ..... 430/96 X  
3,894,868 7/1975 Regensburger ..... 430/96 X  
4,203,764 5/1980 Tosaka et al. ..... 430/67  
4,251,612 2/1981 Chu et al. ..... 430/59

FOREIGN PATENT DOCUMENTS

639318 4/1962 Canada ..... 430/89  
49-135633 12/1974 Japan ..... 430/67

50-50929 5/1975 Japan ..... 430/58  
54-3538 1/1979 Japan ..... 430/67  
1578960 11/1980 United Kingdom .....  
1587312 4/1981 United Kingdom .....

## OTHER PUBLICATIONS

Xerox Disclosure Journal, Band 5, Nr. 2, (Mar.-Apr., 1980).

Research Disclosure, Nr. 109, Article No. 10928, (May, 1973).

Primary Examiner—Roland E. Martin, Jr.  
Attorney, Agent, or Firm—Schwartz, Jeffery, Schwaab, Mack, Blumenthal & Koch

[57] ABSTRACT

An electrophotographic recording material comprising an electrically conductive support, an optional insulating intermediate layer, at least one photoconductive layer comprising a charge carrier generating compound and a charge transporting compound, and a protective transparent cover layer made from a surface abrasion resistant binder composed of a polyurethane resin, polycarbonate resin, phenoxy resin, polyacrylate or polymethacrylate resin, polyurethane formed from a two-component system comprising a polyisocyanate and a hydroxyl group containing polyester or polyether, a polyisocyanate and a hydroxyl group containing acrylic or epoxy resin, polyurethane formed from a one-component system comprising a polyisocyanate prepolymer, or a polyisocyanate having temporarily masked isocyanate groups.

7 Claims, 4 Drawing Figures



FIG. 1



FIG. 2



FIG. 3



FIG. 4



## ELECTROPHOTOGRAPHIC RECORDING MATERIAL WITH ABRASION RESISTANT OVERCOAT

### BACKGROUND OF THE INVENTION

This invention relates to an electrophotographic recording material comprising an electrically conductive support; an optional insulating interlayer; a photoconductive layer comprising at least one charge carrier generating compound and at least one charge transporting compound; and a protective transparent covering layer.

In the electrophotographic process described in U.S. Pat. No. 2,297,691 which is now widely used for preparing electrophotographic copies, thorough cleaning of the photoconductor layer is always required after the toner image developed by a dry method on the photoconductor layer has been transferred to the support of the copy. Usually, cleaning is effected by brushing or wiping the layer with suitable brushes or cloths. In copying machines which utilize fluid developers, the effect of mechanical cleaning is frequently enhanced by also using cleaning fluid. In addition to these cleaning operations, the photoconductive layer is also exposed to other influences which may damage it. For example, it is subject to the action of the dry developer and of the developer station (counter-voltage) and during fluid development, additionally to the action of the developer fluid. It is also exposed to ionized air generated in the charging station. It is known that the requisite cleaning procedures and other influences mentioned result in deterioration of the photoconductor layer, or even in mechanical damage thereto, and thus reduce the service life of the photoconductor.

Recording materials comprising a photoconductive layer comprising at least one layer comprising a charge carrier generating compound and a charge transporting compound are known. For example, German Auslegeschrift 2,314,051 discloses use of highly sensitive, organic photoconductor layers on conductive support films or support bands because of their high elasticity.

In particular, very highly sensitive photoconductor systems, such as those disclosed in German Offenlegungsschrift 2,734,288, can be used in the form of endless bands which, because of their high flexibility, can be passed over guide rollers of relatively small diameter.

Patents such as U.S. Pat. No. 2,901,348, U.S. Pat. No. 4,148,637 and German Offenlegungsschrift 2,452,623 disclose protecting photoconductor layers with an additional covering layer of inorganic or organic materials. A disadvantage of such systems is that they are used either on less flexible layers which are composed of or contain selenium, or on generally less sensitive organic photoconductor systems. Moreover, silane couplers, such as chlorosilane, must be added to these covering layers to improve their stability, or the covering layers additionally contain a photoconductive organic compound.

### SUMMARY OF THE INVENTION

It is the object of the present invention to provide a new electrophotographic recording material.

A further object of the present invention is to provide an electrophotographic recording material which is transparent and highly sensitive.

Another object of the present invention is to provide an electrophotographic recording material having a protective covering layer over the photosensitive material.

5 A still further object of the present invention is to provide an electrophotographic recording material with improved abrasion resistance.

It is also an object of the present invention to provide an electrophotographic recording material which can be developed by a dry method or by a fluid developing recess.

10 An additional object of the present invention is to provide an electrophotographic recording material which has a readily cleanable surface and which resists deterioration during cleaning.

15 Yet another object of the present invention is to provide an electrophotographic recording material which resists both mechanical and chemical deterioration.

20 A further object of the present invention is to provide an electrophotographic recording material with a reduced susceptibility to damage from exposure to ionized air.

25 Another object of the present invention is to provide an electrophotographic recording material having a long service life.

30 A still further object of the present invention is to provide an electrophotographic recording material which can be configured either as a flexible endless band or as a rigid drum.

35 It is also an object of the present invention to provide a multi-layer electrophotographic recording material wherein the various layers adhere well to each other.

Another object of the present invention is to provide an electrophotographic recording material which can effectively utilize organic photoconductive materials.

These and other objects are achieved by providing an electrophotographic recording material wherein the covering layer comprises an abrasion resistant organic binder selected from the group consisting of polyurethane resin, polycarbonate resin, phenoxy resin, polyacrylate or polymethacrylate resin, polyurethane formed from a two-component system comprising a polyisocyanate and a hydroxyl group containing polyester or polyether, a polyisocyanate and a hydroxyl group containing acrylic or epoxy resin, polyurethane formed from a one-component system comprising a polyisocyanate prepolymer, or comprising a polyisocyanate having temporarily masked isocyanate groups. The binders may be non-crosslinking, crosslinkable by subsequent treatment or self-crosslinking.

40 45 50 55 60 65 66 67 68 69 70 71 72 73 74 75 76 77 78 79 80 81 82 83 84 85 86 87 88 89 90 91 92 93 94 95 96 97 98 99 100 101 102 103 104 105 106 107 108 109 110 111 112 113 114 115 116 117 118 119 120 121 122 123 124 125 126 127 128 129 130 131 132 133 134 135 136 137 138 139 140 141 142 143 144 145 146 147 148 149 150 151 152 153 154 155 156 157 158 159 160 161 162 163 164 165 166 167 168 169 170 171 172 173 174 175 176 177 178 179 180 181 182 183 184 185 186 187 188 189 190 191 192 193 194 195 196 197 198 199 200 201 202 203 204 205 206 207 208 209 210 211 212 213 214 215 216 217 218 219 220 221 222 223 224 225 226 227 228 229 230 231 232 233 234 235 236 237 238 239 240 241 242 243 244 245 246 247 248 249 250 251 252 253 254 255 256 257 258 259 260 261 262 263 264 265 266 267 268 269 270 271 272 273 274 275 276 277 278 279 280 281 282 283 284 285 286 287 288 289 290 291 292 293 294 295 296 297 298 299 300 301 302 303 304 305 306 307 308 309 310 311 312 313 314 315 316 317 318 319 320 321 322 323 324 325 326 327 328 329 330 331 332 333 334 335 336 337 338 339 340 341 342 343 344 345 346 347 348 349 350 351 352 353 354 355 356 357 358 359 360 361 362 363 364 365 366 367 368 369 370 371 372 373 374 375 376 377 378 379 380 381 382 383 384 385 386 387 388 389 390 391 392 393 394 395 396 397 398 399 400 401 402 403 404 405 406 407 408 409 410 411 412 413 414 415 416 417 418 419 420 421 422 423 424 425 426 427 428 429 430 431 432 433 434 435 436 437 438 439 440 441 442 443 444 445 446 447 448 449 450 451 452 453 454 455 456 457 458 459 460 461 462 463 464 465 466 467 468 469 470 471 472 473 474 475 476 477 478 479 480 481 482 483 484 485 486 487 488 489 490 491 492 493 494 495 496 497 498 499 500 501 502 503 504 505 506 507 508 509 510 511 512 513 514 515 516 517 518 519 520 521 522 523 524 525 526 527 528 529 530 531 532 533 534 535 536 537 538 539 540 541 542 543 544 545 546 547 548 549 550 551 552 553 554 555 556 557 558 559 560 561 562 563 564 565 566 567 568 569 570 571 572 573 574 575 576 577 578 579 580 581 582 583 584 585 586 587 588 589 5810 5811 5812 5813 5814 5815 5816 5817 5818 5819 5820 5821 5822 5823 5824 5825 5826 5827 5828 5829 5830 5831 5832 5833 5834 5835 5836 5837 5838 5839 5840 5841 5842 5843 5844 5845 5846 5847 5848 5849 5850 5851 5852 5853 5854 5855 5856 5857 5858 5859 5860 5861 5862 5863 5864 5865 5866 5867 5868 5869 58610 58611 58612 58613 58614 58615 58616 58617 58618 58619 58620 58621 58622 58623 58624 58625 58626 58627 58628 58629 58630 58631 58632 58633 58634 58635 58636 58637 58638 58639 58640 58641 58642 58643 58644 58645 58646 58647 58648 58649 58650 58651 58652 58653 58654 58655 58656 58657 58658 58659 58660 58661 58662 58663 58664 58665 58666 58667 58668 58669 58670 58671 58672 58673 58674 58675 58676 58677 58678 58679 58680 58681 58682 58683 58684 58685 58686 58687 58688 58689 58690 58691 58692 58693 58694 58695 58696 58697 58698 58699 586100 586101 586102 586103 586104 586105 586106 586107 586108 586109 586110 586111 586112 586113 586114 586115 586116 586117 586118 586119 586120 586121 586122 586123 586124 586125 586126 586127 586128 586129 586130 586131 586132 586133 586134 586135 586136 586137 586138 586139 586140 586141 586142 586143 586144 586145 586146 586147 586148 586149 586150 586151 586152 586153 586154 586155 586156 586157 586158 586159 586160 586161 586162 586163 586164 586165 586166 586167 586168 586169 586170 586171 586172 586173 586174 586175 586176 586177 586178 586179 586180 586181 586182 586183 586184 586185 586186 586187 586188 586189 586190 586191 586192 586193 586194 586195 586196 586197 586198 586199 586200 586201 586202 586203 586204 586205 586206 586207 586208 586209 586210 586211 586212 586213 586214 586215 586216 586217 586218 586219 586220 586221 586222 586223 586224 586225 586226 586227 586228 586229 586230 586231 586232 586233 586234 586235 586236 586237 586238 586239 586240 586241 586242 586243 586244 586245 586246 586247 586248 586249 586250 586251 586252 586253 586254 586255 586256 586257 586258 586259 586260 586261 586262 586263 586264 586265 586266 586267 586268 586269 586270 586271 586272 586273 586274 586275 586276 586277 586278 586279 586280 586281 586282 586283 586284 586285 586286 586287 586288 586289 586290 586291 586292 586293 586294 586295 586296 586297 586298 586299 586300 586301 586302 586303 586304 586305 586306 586307 586308 586309 586310 586311 586312 586313 586314 586315 586316 586317 586318 586319 586320 586321 586322 586323 586324 586325 586326 586327 586328 586329 586330 586331 586332 586333 586334 586335 586336 586337 586338 586339 586340 586341 586342 586343 586344 586345 586346 586347 586348 586349 586350 586351 586352 586353 586354 586355 586356 586357 586358 586359 586360 586361 586362 586363 586364 586365 586366 586367 586368 586369 586370 586371 586372 586373 586374 586375 586376 586377 586378 586379 586380 586381 586382 586383 586384 586385 586386 586387 586388 586389 586390 586391 586392 586393 586394 586395 586396 586397 586398 586399 586400 586401 586402 586403 586404 586405 586406 586407 586408 586409 586410 586411 586412 586413 586414 586415 586416 586417 586418 586419 586420 586421 586422 586423 586424 586425 586426 586427 586428 586429 586430 586431 586432 586433 586434 586435 586436 586437 586438 586439 586440 586441 586442 586443 586444 586445 586446 586447 586448 586449 586450 586451 586452 586453 586454 586455 586456 586457 586458 586459 586460 586461 586462 586463 586464 586465 586466 586467 586468 586469 586470 586471 586472 586473 586474 586475 586476 586477 586478 586479 586480 586481 586482 586483 586484 586485 586486 586487 586488 586489 586490 586491 586492 586493 586494 586495 586496 586497 586498 586499 586500 586501 586502 586503 586504 586505 586506 586507 586508 586509 586510 586511 586512 586513 586514 586515 586516 586517 586518 586519 586520 586521 586522 586523 586524 586525 586526 586527 586528 586529 586530 586531 586532 586533 586534 586535 586536 586537 586538 586539 586540 586541 586542 586543 586544 586545 586546 586547 586548 586549 586550 586551 586552 586553 586554 586555 586556 586557 586558 586559 586560 586561 586562 586563 586564 586565 586566 586567 586568 586569 586570 586571 586572 586573 586574 586575 586576 586577 586578 586579 586580 586581 586582 586583 586584 586585 586586 586587 586588 586589 586590 586591 586592 586593 586594 586595 586596 586597 586598 586599 586600 586601 586602 586603 586604 586605 586606 586607 586608 586609 586610 586611 586612 586613 586614 586615 586616 586617 586618 586619 586620 586621 586622 586623 586624 586625 586626 586627 586628 586629 586630 586631 586632 586633 586634 586635 586636 586637 586638 586639 586640 586641 586642 586643 586644 586645 586646 586647 586648 586649 586650 586651 586652 586653 586654 586655 586656 586657 586658 586659 586660 586661 586662 586663 586664 586665 586666 586667 586668 586669 586670 586671 586672 586673 586674 586675 586676 586677 586678 586679 586680 586681 586682 586683 586684 586685 586686 586687 586688 586689 586690 586691 586692 586693 586694 586695 586696 586697 586698 586699 586700 586701 586702 586703 586704 586705 586706 586707 586708 586709 586710 586711 586712 586713 586714 586715 586716 586717 586718 586719 586720 586721 586722 586723 586724 586725 586726 586727 586728 586729 586730 586731 586732 586733 586734 586735 586736 586737 586738 586739 586740 586741 586742 586743 586744 586745 586746 586747 586748 586749 586750 586751 586752 586753 586754 586755 586756 586757 586758 586759 586760 586761 586762 586763 586764 586765 586766 586767 586768 586769 586770 586771 586772 586773 586774 586775 586776 586777 586778 586779 586780 586781 586782 586783 586784 586785 586786 586787 586788 586789 586790 586791 586792 586793 586794 586795 586796 586797 586798 586799 586800 586801 586802 586803 586804 586805 586806 586807 586808 586809 586810 586811 586812 586813 586814 586815 586816 586817 586818 586819 586820 586821 586822 586823 586824 586825 586826 586827 586828 586829 586830 586831 586832 586833 586834 586835 586836 586837 586838 586839 586840 586841 586842 586843 586844 586845 586846 586847 586848 586849 586850 586851 586852 586853 586854 586855 586856 586857 586858 586859 586860 586861 586862 586863 586864 586865 586866 586867 586868 586869 586870 586871 586872 586873 586874 586875 586876 586877 586878 586879 586880 586881 586882 586883 586884 586885 586886 586887 586888 586889 586890 586891 586892 586893 586894 586895 586896 586897 586898 586899 586900 586901 586902 586903 586904 586905 586906 586907 586908 586909 586910 586911 586912 586913 586914 586915 586916 586917 586918 586919 586920 586921 586922 586923 586924 586925 586926 586927 586928 586929 586930 586931 586932 586933 586934 586935 586936 586937 586938 586939 586940 586941 586942 586943 586944 586945 586946 586947 586948 586949 586950 586951 586952 586953 586954 586955 586956 586957 586958 586959 586960 586961 586962 586963 586964 586965 586966 586967 586968 586969 586970 586971 586972 586973 586974 586975 586976 586977 586978 586979 586980 586981 586982 586983 586984 586985 586986 586987 586988 586989 586990 586991 586992 586993 586994 586995 586996 586997 586998 586999 586100 586101 586102 586103 586104 586105 586106 586107 586108 586109 586110 586111 586112 586113 586114 586115 586116 586117 586118 586119 586120 586121 586122 586123 586124 586125 586126 586127 586128 586129 586130 586131 586132 586133 58

FIG. 1 is a schematic sectional view of an electrophotographic recording material according to the invention comprising a single photoconductive layer;

FIG. 2 is a schematic sectional view of an alternate embodiment of electrophotographic recording material comprising a two layer photoconductor arrangement;

FIG. 3 is a schematic sectional view of a third electrophotographic recording material which is provided with an insulating interlayer; and

FIG. 4 is a schematic sectional view of an electrophotographic recording material embodiment including a layer comprising a dispersed charge-generating compound.

#### DETAILED DESCRIPTION OF PREFERRED EMBODIMENTS

The electrophotographic recording material according to the invention is schematically represented by the attached FIGS. 1 to 4. As illustrated in FIG. 1, the photoconductive layer can take the form of a single layer, as indicated by reference numeral 6. It can also take the form of a two layer arrangement as depicted in FIGS. 2 and 3, comprising a layer 2 containing compounds which generate charge carriers and a layer 3 containing compounds which transport charges. In general, the two layer arrangement is preferred. The conductive support is identified by reference numeral 1 in each case. An insulating interlayer is designated by reference numeral 4. Reference numeral 5 identifies a layer containing a charge carrier generating compound in dispersion. The numeral 7 indicates a protective covering layer according to the invention.

Examples of suitable conductive supports include aluminum foil, and polyester films which may be transparent and on which aluminum has been vapor-deposited or which are laminated to aluminum. Any other support which has been rendered sufficiently conductive can also be used.

The insulating interlayer may comprise an alumina layer which may be produced thermally, anodically (electrochemically) or chemically. Alternately, the insulating layer can also be composed of organic materials. Different natural resin binders or synthetic resin binders which have good adhesion to an aluminum or other metal surface and suffer little incipient dissolution when further layers are subsequently applied, may be used. Suitable resins include polyamide resins, polyvinylphosphonic acid, polyurethanes, polyester resins, or specifically alkali-soluble binders such as styrene/maleic anhydride copolymers. The thickness of organic interlayers of this type can be up to 5  $\mu\text{m}$ . When an alumina layer is used, the thickness of the layer lies in most cases in the range from 0.01–1  $\mu\text{m}$ .

The layers 2 and 5 are charge carrier generating layers. The compounds which are used here and generate charge carriers determine, to a particular degree, spectral light-sensitivity of the photoconductive system. Many different types of dyestuffs can be employed as charge carrier generating substances. Useful charge carrier generating substances include perylene-3,4,9,10-tetracarboxylic acid anhydride or perylene-3,4,9,10-tetracarboxylic acid imide derivatives according to German Offenlegungsschrift 22 37 539; N,N'-bis-(3-methoxy propyl)-3,4,9,10-perylene tetracarboxylic acid imide according to German Pat. No. 22 32 513; polynuclear quinones according to German Offenlegungsschrift 22 37 678; cis- or transperinones according to German Offenlegungsschrift 22 39 923; thioindigo dye-

stuffs according to German Offenlegungsschrift 22 37 680; quinacridones according to German Offenlegungsschrift 22 37 679; condensation products of benzo-4,10-thioxanthene-3,1'-dicarboxylic acid anhydride and amines according to German Offenlegungsschrift 23 55 075; phthalocyanine derivatives according to German Offenlegungsschrift 22 39 924; and dyestuffs which in accordance with the procedure described in *Bull. Chem. Soc. Japan*, Vol. 25, pp. 411–413 (1952) are produced by condensation from perylene-3,4,9,10-tetracarboxylic acid anhydride and o-phenylene diamine or 1,8-diaminophthaline, according to German Offenlegungsschrift 23 14 051. Furthermore, dyestuffs according to German Offenlegungsschriften 22 46 255, 23 53 639 and 23 56 370 may also be used.

As already mentioned above, thin layers of inorganic materials which generate charge carriers are also suitable. Such layers may be produced by vapor-depositing selenium, doped selenium, cadmium sulfide, and similar photosensitive materials.

A homogeneous, closely packed layer 2 is preferably applied by vapor-deposition in vacuo. Advantageously, the thickness of the layer 2 will range between about 0.005 and 3  $\mu\text{m}$ . The adhesive strength and homogeneity of the vapor-deposited layer are particularly favorable within this range.

In combination with the interlayer, or as a substitute for the interlayer, homogeneous, well covering dye layers having thicknesses on the order of magnitude of 0.1 to 3  $\mu\text{m}$  can also be prepared by milling or grinding the dye with a binder, especially with highly viscous cellulose nitrates and/or crosslinking binder systems such as acrylic resins which can be crosslinked by polyisocyanate, or lacquers formed from polyisocyanates and hydroxyl group containing polyesters or polyethers. The resulting dye dispersions 5 are subsequently applied to the support 1 as shown in FIG. 4. Organic compounds which have an extended  $\pi$ -electron system are most suitable as the charge transport material in layers 3 or 6. These include, in particular, monomeric aromatic or heterocyclic compounds, such as those which contain at least one dialkylamino group or two alkoxy groups. The oxadiazole derivatives mentioned in German Pat. No. 1,058,836 have proved suitable, particularly 2,5-bis-(p-diethylaminophenyl)-1,3,4-oxadiazole. Further examples of suitable monomeric electron donor compounds are triphenylamine derivatives; highly condensed aromatic compounds such as pyrene; benzo-condensed heterocyclic compounds; pyrazoline derivatives or imidazole derivatives as disclosed in German Pat. Nos. 1,060,714, and 1,106,599; triazole derivatives, thiadiazole derivatives and especially oxazole derivatives, for example 2-phenyl-4-(2-chlorophenyl)-5-(4-diethylamino)-oxazole, as disclosed in German Pat. Nos. 1,060,260, 1,299,296 and 1,120,875.

The charge-transport layer 3 has virtually no photosensitivity in the visible range (420–750 nm). Preferably, it is composed of a mixture of an electron donor compound with a resin binder, if a negative charge is to be obtained.

Layer 3 is preferably transparent. It is also possible, however, that in a case such as a transparent conductive support, it would not need to be transparent. The layer has a high electrical resistance ( $\geq 10^{12} \Omega$ ), and in the dark it prevents leakage or discharge of the electrostatic charge. When exposed to light, it transports the charges generated in the organic dye layer.

In addition to the previously described compounds which generate and transport charge carriers, the added binder affects both the mechanical properties, such as abrasion resistance, flexibility, film-forming, etc., and to a certain extent the electrophotographic properties, such as photosensitivity, residual charge and cyclical behavior.

The binders employed are film-forming compounds, such as polyester resins, polyvinyl chloride/polyvinyl acetate copolymers, styrene/maleic anhydride copolymers, polycarbonates, silicone resins, polyurethanes, epoxy resins, acrylates, polyvinyl acetals, polystyrenes, cellulose derivatives such as cellulose acetobutyrate, and the like. Moreover, subsequently crosslinkable binder systems such as DD lacquers (for example Desmophen/Demodur®, Bayer AG), acrylate resins which can be crosslinked by polyisocyanate, melamine resins, unsaturated polyester resins and the like, may be used successfully.

Because of the combined advantages (high photosensitivity, flash sensitivity, high flexibility), the use of cellulose nitrates, particularly the high-viscosity types, is preferred.

The mixing ratio of the charge transporting compound to the binder may vary. However, relatively strict limits are posed by the requirement for maximum photosensitivity, i.e., the greatest possible proportion of charge transporting compound, and the simultaneous requirement that crystallization of the charge transporting compound be prevented and that the flexibility of the layer be increased, i.e., the greatest possible proportion of binder. In general, a mixing ratio of about 1:1 parts by weight has proved to be preferable, but ratios between 4:1 and 1:2 are also suitable. The thickness of the phototransport layer 3 or 6 lies preferably between about 3 and about 20  $\mu\text{m}$ .

Conventional additives may be added to the layer including flow agents such as silicone oils; wetting agents, particularly non-ionic substances; and plasticizers of varying composition such as those based on chlorinated hydrocarbons or on phthalates. If desired, sensitizers and/or acceptors can also be included as additives to the charge transport layer, but only to such an extent that the optical transparency of the charge transport layer is not significantly impaired.

In conjunction with the covering layer according to the invention, additions of micronized organic or inorganic powders in quantities of up to about 30% by weight, preferably about 10% by weight, have also proved advantageous. In this way, the abrasion resistance is improved to a certain extent, and, the adhesion of the subsequently applied covering layer is markedly improved by the rougher, dull surface. Preferred organic powders include micronized polypropylene waxes, polyethylene waxes, polyamide waxes or powders of polytetrafluoroethylene or polyvinylidene fluoride. Useful inorganic powders include those based on silica.

Either non-crosslinking binders, subsequently crosslinkable binders, or self-crosslinking binders can be used as the organic binders resistant to surface abrasion.

Polyurethane resins, polycarbonate resins, phenoxy resins, polyacrylates or polymethacrylates may be mentioned as non-crosslinking organic binders. Such resins can be used individually or in mixtures. Preferably, aromatic or aliphatic, non-reactive, linear polyurethanes or a binder obtained from dihydroxydiphenylal-

kane and phosgene are used. Polysulfones, polyphenylene oxides and polyvinyl acetates are also suitable.

Suitable subsequently crosslinkable binders include two-component systems comprising saturated or unsaturated polyesters or polyethers containing hydroxyl groups which crosslink with an aliphatic and/or aromatic polyisocyanate resin, or acrylic or epoxy resins which contain hydroxyl groups and crosslink with polyisocyanate. Useful one-component systems include moisture-curing polyisocyanate prepolymers, air-drying polyurethane resins (polyurethane alkyd resins), or temporarily masked polyisocyanates having isocyanate groups capable of crosslinking on heating.

Suitable self-crosslinking binders, which optionally may be heat-curable, include pure acrylic resins, preferably aqueous dispersions; or heat-curable acrylic resins which crosslink by external action, if desired with an addition of melamine resin. Epoxy resin systems with hardeners, as well as unsaturated heat-curing polyester resins with or without an accelerator, can also be used successfully.

It has also proved to be advantageous for the covering layer to comprise a self-crosslinking polyisocyanate and the photoconductive layer to comprise a compound with hydroxyl groups.

The aforementioned organic binders are outstandingly suitable for the protective covering layer 7 because of their homogeneous film formation and flexibility, their abrasion resistance and possible application methods. The influence of such layers on the photosensitivity of the recording material is negligibly small.

Thin applications of such protective covering layers are optically transparent. The preferred coherent layer produced on an organic photoconductor in a two-layer arrangement has a uniform thickness of about 0.5 to about 10  $\mu\text{m}$ , preferably from about 0.5 to about 5.0  $\mu\text{m}$ . Film surfaces are smooth, which is necessary for optimum cleaning. The adhesion between the covering layer and the photoconductor system is also sufficient to withstand mechanical stresses such as those due to the action of a cleaning brush. Compared with the photoconductor system to be coated, the abrasion resistance is markedly improved. It is important that the triboelectric behavior of the covering layer be the same as that of the photoconductor layer. At a storage temperature of 40°–50° C., the covering layer is not tacky, and there is also no migration of any component out of the photoconductor layer. The covering layer also serves to prevent crystallization effects which can be induced by contact with the photoconductor surface. The electrical conductivity of the covering layer is small enough that it does not affect the charging capacity of the photoconductor. On the other hand, the materials provide the covering layer with electrical permeability so that upon exposure to light, charges can leak away from the surface—down to a small residual voltage in some cases. The electrostatic charge image remains fully preserved after exposure until the image is developed, and this is necessary, since otherwise the resolution of the copy deteriorates. The specific electrical resistance is not altered by the moisture content of the surroundings. Finally, the film surface is free from hydrophilic components, so that the surface resistivity is not altered by climatic conditions.

The preferred systems for applying the coating are coating on a spreading machine for applying the coating to substrates such as photoconductor bands, preferably by continuous application, as well as spraying tech-

niques, including if desired electrostatic techniques for applying the covering layer to substrates such as drums. Also, if drums are dip-coated, care must be taken as a restriction, that the photoconductor system is stable and will not dissolve during subsequent dip-coating with cover layer materials.

In a particular embodiment of the recording material according to the invention, additions of micronized organic or inorganic powders are dispersed in the photoconductive layer, whereby the adhesion-promotion and the abrasion properties are markedly improved.

In a further embodiment, photoconductive layers comprising, for example, hydroxyl group containing binders, particularly cellulose esters such as cellulose nitrates, are coated with a polyfunctional aromatic/aliphatic polyisocyanate or polyisocyanate prepolymer, and an adhesion-promoting, hardened transition zone is thus formed between the photoconductive layer and the covering layer.

The invention will be explained in greater detail with reference to the following non-limiting examples.

#### EXAMPLE 1

Solutions of an abrasion-resistant binder from the following Table I are applied, by continuous flow techniques and immediately thereafter dried for 5 minutes, onto two layer photoconductors which are built up, in the following order from an electrically conductive support comprising a 75  $\mu\text{m}$  thick polyester film on which aluminum has been vapor deposited; a vapor-deposited layer of N,N'-dimethylperylimide (C. I. 71,129); and a charge-transport layer comprising 2,5-bis-(4-diethylaminophenyl)-1,3,4-oxadiazole (To) and highly viscous cellulose nitrate in a weight ratio of 65:35. The thicknesses of the individual protective covering layers with the different binders lie in the range of  $2 \pm 0.5 \mu\text{m}$ . Both the photosensitivity and the abrasion resistance properties of the material with and without covering layer are tested under identical conditions. The results are summarized in the following Table I.

The measurement of the photosensitivity is carried out as follows. To determine the discharge curves in light, a test sample is moved on a rotating disk through a charging device to an exposure station, where it is continuously exposed with a xenon lamp. A heat-absorbing glass and a neutral filter having a transparency of 15% are placed in front of the xenon lamp. The light intensity in the plane of measurement lies in the range of 40-60  $\mu\text{W}/\text{cm}^2$ , and is measured with an optometer immediately after the light discharge curve has been determined. The charge level ( $U_o$ ) and the photo-induced decay curve in light are recorded oscilloscopically through a transparent probe via an electrometer. The photoconductor layer is characterized by the charge level ( $U_o$ ) and the time ( $T_{1/2}$ ), after which half the charge ( $U_o/2$ ) is reached. The product of  $T_{1/2}$  and the measured light intensity  $I$  ( $\mu\text{W}/\text{cm}^2$ ) is the half-value energy  $E_{1/2}$  ( $\mu\text{J}/\text{cm}^2$ ). The residual charge ( $U_R$ ) after 0.1 second, determined from the above discharge curves in light, is a further measure of the discharge of the photoconductor layer.

To test the abrasion resistance properties, the abrasion of the various materials (photoconductor and cover layers) is measured on a standard abrasion test apparatus (Type 352 Taber Abraser) under the following conditions:

|                                       |                    |
|---------------------------------------|--------------------|
| Abrasive Material (friction rollers): | CS-10 F Calibrese  |
| Loading:                              | 250 g              |
| Abrasion area:                        | 26.3 $\text{cm}^2$ |
| Number of cycles:                     | 200                |

The abrasion in  $\text{g}/\text{m}^2$  is determined by dividing the gravimetrically determined abrasion in mg by the abrasion area.

TABLE I

| Protective covering layer                                                                            | Thickness g/m <sup>2</sup> | (-) $U_o/V$ | $E_{1/2}(\mu\text{J}/\text{cm}^2)$ | $U_R/V$ after 0.1 second | Abrasion loss g/m <sup>2</sup>         |
|------------------------------------------------------------------------------------------------------|----------------------------|-------------|------------------------------------|--------------------------|----------------------------------------|
| None                                                                                                 | 0                          | 580         | 1.1                                | 105                      | 2.2-2.5                                |
| Polyvinyl acetate dispersion in water                                                                | 1.6                        | 480         | 1.2                                | 105                      | 1.6                                    |
| <u>Polyurethane</u><br>(crosslinking subsequently)                                                   |                            |             |                                    |                          |                                        |
| 1.2 parts of polyisocyanate (75%), 1 part of polyester and 0.1%, relative to solids, of zinc octoate | 2.5                        | 535         | 1.4                                | 125                      | $\leq 0.01$<br>(drying for 30 minutes) |
| Aromatic, non-reactive linear polyurethane                                                           | 2-2.5                      | 520         | 1.1                                | 100                      | 0.01                                   |
| <u>Epoxide resin</u><br>(reactive)                                                                   |                            |             |                                    |                          |                                        |
| Poly-aminoamide adduct, Eurepox 716 epoxide resin 1:1                                                | 1.8                        | 570         | 2.0                                | 195                      | 1.3                                    |
| Phenoxy resin                                                                                        | 2.0                        | 555         | 1.2                                | 125                      | 0.2-0.05                               |

#### EXAMPLE 2

45 A photoconductive system, as described in Example 1, but containing 50 parts by weight of To, 25 parts by weight of a polyester resin and 25 parts by weight of a polyvinyl chloride/polyvinyl acetate copolymer having a thickness of about 10  $\mu\text{m}$ , is coated with an aqueous polyacrylate dispersion (4% acrylate/styrene copolymer in  $\text{H}_2\text{O}$ ) by continuous application in a single machine-coat. After drying, the thickness of this protective covering layer is about 0.5  $\mu\text{m}$ . While the photosensitivity remains the same, the abrasion resistance is improved and the shelf-life is increased by the applied shiny layer.

50 The values in the following Table II are determined in the same manner as in Example 1:

TABLE II

| Covering layer | Thickness g/m <sup>2</sup> | (-) $U_o/V$ | $E_{1/2}(\mu\text{J}/\text{cm}^2)$ | $U_R/V$ after 0.1 second | Abrasion loss g/m <sup>2</sup> |
|----------------|----------------------------|-------------|------------------------------------|--------------------------|--------------------------------|
| None           | 0                          | 750         | 3.5                                | 225                      | 2.1                            |
| Polyacrylate   | 0.4                        | 750         | 3.3                                | 205                      | 1.6                            |

## EXAMPLE 3

The surface properties and photosensitivity of a photoconductive system produced according to Example 2 were tested in a dry toner copying apparatus. A magnetic brush device with a two-component toner mixture is used for development, and the layer is moved past a rotating brush for cleaning residual toner from the photoconductor surface. It is found thereby that the quality of the copies is the same under identical copying conditions with and without a covering layer. In a long-term copying test, strong surface films were apparent after 5,000 copies on the photoconductor layer without a protective covering layer, and the surface is duller. In contrast thereto, only insignificant surface films are 15 discernible on the system provided with a covering layer, and the surface is still shiny.

## EXAMPLE 4

To improve the abrasion resistance properties, 5% by 20 weight, based on solids content, of micronized polyethylene wax (PE) or micronized polytetrafluoroethylene (PTFE) are dispersed into a charge-transport layer composed of 65 parts of To and 35 parts of cellulose nitrate. A dull, homogeneous photoconductor layer is obtained by subsequently coating the dispersion onto an aluminum/polyester support, on which N,N'-dimethyl- 25 perylimide has been vapor deposited. The photosensitivity and abrasion are determined in accordance with the procedures of Example 1. Results are shown in the 30 following Table III:

TABLE III

| Addition<br>(5%) | Layer<br>weight<br>g/m <sup>2</sup> | Layer<br>(—)U <sub>o</sub> /V | U <sub>R</sub> /V<br>after<br>0.1<br>second | Abrasion<br>loss<br>g/m <sup>2</sup> |
|------------------|-------------------------------------|-------------------------------|---------------------------------------------|--------------------------------------|
| None             | about                               | 530                           | 1.8                                         | 55 2.2-2.5                           |
| PTFE             | 8                                   | 640                           | 2.0                                         | 100 1.7                              |
| PE               | 7.9                                 | 650                           | 1.9                                         | 110 1.3-1.6                          |

## EXAMPLE 5

An aqueous dispersion of self-crosslinking, heat-curable, pure acrylic resin is applied about 2  $\mu\text{m}$  thick to the 45 photoconductor layers described in Example 4, with and without the micronized powder addition, and the resulting covers are dried for about 10 minutes at 110° C. in a circulating air oven.

The homogeneous products are subjected to an abrasion test according to Example 1, and the results are:

|                                            |                       |
|--------------------------------------------|-----------------------|
| Photoconductor layer + covering layer      | 0.95 g/m <sup>2</sup> |
| Photoconductor layer + PE + covering layer | 0.5 g/m <sup>2</sup>  |

This shows that additions of a micronized powder, in particular in combination with covering layers, give a marked reduction in abrasion.

## EXAMPLE 6

Various polycarbonate binders (I. Makrolon 2504®, Bayer AG; and II. Lexan 141®, General Electric) and a polysulfone (Polysulfone 1700® Union Carbide) show a very good abrasion resistance, when being whirled coated onto a 100  $\mu\text{m}$  thick aluminum foil and dried for about 5 minutes at 110° C. The abrasion loss is

determined according to the procedure of Example 1 to be:

|   |                  |                       |
|---|------------------|-----------------------|
| 5 | Polycarbonate I  | 0.01 g/m <sup>2</sup> |
|   | Polycarbonate II | 0.01 g/m <sup>2</sup> |
|   | Polysulfone      | 0.15 g/m <sup>2</sup> |

A solution of polycarbonate I in tetrahydrofuran is 10 applied by continuous application machine coating about 2  $\mu\text{m}$  thick onto a photoconductor layer as described in Example 1. After drying, an abrasion of 0.04 g/m<sup>2</sup> is measured.

The foregoing embodiments have been set forth as illustrations of the invention and are not intended to be limiting. Since modifications of the disclosed embodiments may occur to persons skilled in the art, the scope of the invention should be limited solely by the appended claims and equivalents.

I claim:

1. An electrophotographic recording material comprising an electrically conductive support, a photoconductive layer containing at least one organic charge carrier generating compound and at least one organic charge transporting compound, and a protective transparent covering layer having a thickness in the range from about 0.5 to about 10  $\mu\text{m}$  and comprising a surface abrasion resistant subsequently crosslinkable material, said abrasion resistant material being a two-component system comprising a polyisocyanate selected from the group consisting of aliphatic polyisocyanates and aromatic polyisocyanates and a cross-linking, hydroxyl group containing compound selected from the group consisting of saturated polyesters, saturated polyethers, acrylic resins and epoxy resins.

2. An electrophotographic recording material comprising an electrically conductive support, a photoconductive layer containing at least one organic charge carrier generating compound and at least one organic charge transporting compound, and a protective transparent covering layer having a thickness in the range from about 0.5 to about 10  $\mu\text{m}$  and comprising a surface abrasion resistant subsequently crosslinkable material, wherein the covering layer comprises a self-crosslinking polyisocyanate and the photoconductive layer comprises a compound containing hydroxyl groups.

3. A recording material according to claim 1 or 2, wherein a finely micronized powder is dispersed in the photoconductive layer.

4. A recording material according to claim 3, wherein the micronized powder is selected from the group consisting of polypropylene wax, polyethylene wax, polyamide wax, polytetrafluoroethylene powder, polyvinylidene fluoride powder, and micronized silica.

5. A recording material according to claim 1 or 2 further comprising an insulating interlayer interposed between said conductive support and said photoconductive layer.

6. A recording material according to claim 1 or 2, wherein said photoconductive layer further comprises an organic resin binder.

7. A recording material according to claim 1 or 2, wherein said photoconductive layer comprises two sublayers, one of said sublayers containing said charge carrier generating compound and the other of said sublayers containing said charge transporting compound.

\* \* \* \* \*